# EUROPEAN PATENT SPECIFICATION

(11) **EP 1 274 818 B1**
(45) Date of publication and mention of the grant of the patent: **31.05.2006**
(21) Application number: 01920806.5
(22) Date of filing: 08.02.2001
(51) Int. Cl.: C10L 1/06, C10L 1/08

(54) **USE OF DI-ISOBUTYLENE IN A FUEL COMPOSITION**
VERWENDUNG DI-ISOBUTENS IN EINER BRENNSTOFFZUSAMMENSETZUNG
UTILISATION DU DI-ISOBUTYLENE DANS UNE COMPOSITION DE CARBURANT

(30) Priority: 14.02.2000 GB 0003386
(43) Date of publication of application: 15.01.2003
(73) Proprietor: ExxonMobil Research and Engineering Company, Annandale, NJ 08801 (US)
(72) Inventor: PACE, Stuart, Winchester HANTS. SO22 5DY (GB); SCHILOWITZ, Alan, Mark, Highland Park, NJ 08904 (US)
(74) Representative: Dew, Melvyn John
(86) International application number: PCT/US2001/009792
(87) International publication number: WO 2001/060955

(56) References cited:
- DATABASE WPI Section Ch, Week 199621 Derwent Publications Ltd., London, GB; Class E17, AN 1996-205833 XP002171159 & JP 08 073870 A (TONEN CORP), 19 March 1996 (1996-03-19) cited in the application

## Description

This invention relates to fuel compositions comprising an anti-foam additive to reduce the time needed to break up any foam formation during the filling of a vehicle's fuel tank thereby enabling a more complete filling of the tank and at the same time reducing risk of spillage.

The problem of foaming of fuels due to entrainment of air during filling of fuel tanks of vehicles is well known. The problem has hitherto been mitigated by adding to the fuel antifoams which are substantially non-hydrocarbonaceous. An example of such a non-hydrocarbonaceous additive is a silicon containing polymer. Non-hydrocarbonaceous additives usually have to undergo a rigorous testing programme with respect to their compatibility with the fuel and also environmental considerations. However, if the additive is a hydrocarbon, especially a non-aromatic hydrocarbon, the issues of compatibility and environmental considerations are not as critical. JP-A-08073870 discloses gasoline compositions for two-cycle engines which contain at least 10 vol % 7-8C olefinic hydrocarbons and have a Tso of 93-105°C, a final distillation temperature of 110-150°C and an octane No. by the motor method of at least 95. Amongst the 11 olefins listed is mentioned 2,4,4-trimethyl-1-pentene. However, it is not clear whether these olefins are used as a blend of several. In any event, the olefins are not used as anti-foaming agents but to achieve high output and low fuel consumption and to avoid seizure even at high compression ratios. Moreover, gasoline used in two-cycle engines (ie two-stroke engines) inevitably have lubricating oils admixed therewith and hence are not as susceptible to foaming as gasolines free of such lubricating oils.

Similarly, SAE Paper 950740 describes various compounds being added to a mixture of toluene (boiling point about 110°C) and isooctane (boiling point 99°C) to monitor the emissions of vehicles powered therewith. One such compound added is di-isobutylene in an amount > 15% by volume. The resultant mixture is unlikely to have a final boiling point above 150°C and there is no mention of the use of di-isobutylene as an anti-foam in this document.

Similarly, JP-A-06200263 describes a composition which contains at least 65% by volume based on the total base fuel of a high boiling component with a boiling point from 80-120°C which uses 7-8C paraffin type or olefin type hydrocarbon. The abstract of this patent makes no mention of any other base fuels or specific olefins in this range and there is no mention of any of such olefins as anti-foaming agents.

WO 99/49003 discloses gasoline formulations which contain, *inter alia,* at least 5% by volume of saturated C₇/C₈ branched chain hydrocarbons. In any event, there is no mention of the use of these as anti-foaming agents.

It is an object of the present invention to formulate fuel compositions wherein an anti-foam which is an unsaturated, non-aromatic hydrocarbon is used which is capable of reducing the break-up time to disperse any such foams formed.

The present invention provides the use of di-isobutylene as an anti-foam for a base fuel as defined in claim 1 of the set of claims following this description. Optional and/or preferred features of the invention are defined in the other claims in the set of claims following this description.

The base fuels may comprise mixtures of saturated, olefinic, and aromatic hydrocarbons, and these can be derived from straight run streams, thermally or catalytically cracked hydrocarbon feedstocks, hydrocracked petroleum fractions, catalytically reformed hydrocarbons, or synthetically produced hydrocarbon mixtures. The present invention is particularly applicable to a broad range of petroleum fuels from the light boiling gasoline (which typically boils between 50 and 200°C) to distillate fuel (which typically boils between 150 and 400°C). The most common distillate fuels suitable for use in the present invention as base fuels are selected from motor gasoline, kerosene and diesel fuels. The sulfur content of the base fuel is suitably less than100 ppm by weight, preferably less than 50 ppm by weight and more preferably less than 30 ppm by weight. Such low sulfur levels can be achieved in a number of ways. For instance, this may be achieved by well known methods such as, e.g., catalytic hydrodesulfurization.

Di-isobutylene used as an anti-foam in accordance with the use of the invention is employed in an amount greater than 2.5% by volume based on the total fuel composition, suitably up to 35% by volume, preferably less than 15% by volume, more preferably from 5.0 to less than 15% by volume, still more preferably from 7.5% to less than 15% by volume of the total fuel composition.

Di-isobutylene can readily be obtained by dimerization of isobutylene. It is generally prepared from a crude mixture of olefins and usually contains a mixture of various C₈-olefin isomers but always comprises 2,4,4-trimethylpent-1-ene admixed with 2,4,4-trimethylpent-2-ene. These two isomers are suitably present in the di-isobutylene in a weight ratio of about 75% (-1-ene) to about 25% (-2-ene).

Di-isobutylene has an advantage over other non-hydrocarbonaceous anti-foams such as silicon based polymers in that di-isobutylene is substantially miscible with conventional fuels in all proportions. Di-isobutylene has the further advantage that current plants making methyl tert-butyl ether (hereafter "MTBE") from isobutylene and methanol (MTBE having more recently fallen out of favour upon environmental considerations), can be readily switched to convert the same isobutylene feedstock to di-isobutylene. Furthermore, di-isobutylene can readily make up the additional component volume to replace the MTBE used hitherto in automotive fuel component pool.

It has also been found that the reduction in break-up time for foams formed is not due to a dilution effect of di-isobutylene. Test results show that addition of up to 2.5% by volume of di-isobutylene in the fuel did not show any reduction in the foam break-up time of the fuel tested.

The present invention is further illustrated with reference to the following Examples:

Tests were carried out in which di-isobutylene (a mixture of 3 parts 2,4,4-trimethylpent-1-ene and 1 part 2,4,4-trimethylpent-2-ene) was added to varying quantities to a distillate fuel which was susceptible to foam formation. The resultant admixture was tested in the BNPe Anti-Foam test (French Standard Test NF M 07-075) and the results obtained are shown in Table 1 below:

**TABLE 1**

| **Blend** | **Fuel (ml)** | **DIB (ml)** | **DIB (%)** | **Foam Vol (ml)** | | **Mean Value** | **Break-up Time (seconds)** | | **Mean Value** |
|---|---|---|---|---|---|---|---|---|---|
| 1 | 300 | 0 | 0 | 126 | 124 | 125 | 79.2 | 82.5 | 80.9 |
| 2 | 292.5 | 7.5 | 2.5 | 130 | 128 | 129 | 79.7 | 81 | 80.4 |
| 3 | 285 | 15 | 5 | 130 | 132 | 131 | 62.3 | 66.9 | 64.6 |
| 4 | 270 | 30 | 10 | 142 | 140 | 141 | 51.9 | 49.6 | 50.8 |

| | | | | | | | | | |
|---|---|---|---|---|---|---|---|---|---|
| DIB - Di-isobutylene (a mixture of 3 parts 2,4,4-trimethylpent-1-ene and 1 part 2,4,4-trimethylpent-2-ene) | | | | | | | | | |

## Claims

1. The use of di-isobutylene as an anti-foam for a base fuel having a final boiling point greater than 150°C wherein the di-isobutylene comprises greater than 2.5 % by volume based on the total fuel composition.

2. The use of claim 1 wherein the di-isobutylene comprises less than 15% by volume of the total fuel composition.

3. The use of claim 1 or claim 2 wherein the di-isobutylene comprises from 5% to less than 15% by volume of the total fuel composition.

4. The use of any preceding claim wherein the di-isobutylene comprises a mixture of 2,4,4-trimethylpent-1-ene and 2,4,4-trimethylpent-2-ene.

5. The use of any preceding claim wherein the di-isobutylene comprises a mixture of 2,4,4-trimethylpent-1-ene and 2,4,4-trimethylpent-2-ene in a ratio of about 75% to about 25% by weight.

6. The use of any preceding claim wherein the base fuel comprises mixtures of saturated, olefinic and aromatic hydrocarbons derivable from straight run streams, thermally or catalytically cracked hydrocarbon feedstocks, hydrocracked petroleum fractions, catalytically reformed hydrocarbons, or synthetically produced hydrocarbon mixtures.

7. The use of any preceding claim wherein the base fuel is a petroleum fuel having a boiling range from gasoline (which typically boils in the range of from 50 to 200°C with a final boiling point exceeding 150°C) to distillate fuel (which typically boils between 150 and 400°C).

8. The use of any preceding claim wherein the base fuel is a common distillate fuel selected from motor gasoline, kerosene and diesel fuels.

9. The use of any preceding claim wherein the base fuel has a sulfur content of less than 100ppm by weight.

10. The use of any preceding claim wherein the base fuel has a sulfur content of less than 50 ppm by weight.

## Patentansprüche

1. Verwendung von Diisobutylen als Antischaummittel für einen Basiskraftstoff mit einem Endsiedepunkt von mehr als 150 °C, bei der das Diisobutylen bezogen auf die gesamte Kraftstoffzusammensetzung mehr als 2,5 Vol.% ausmacht.

2. Verwendung nach Anspruch 1, bei der das Diisobutylen weniger als 15 Vol.% der gesamten Kraftstoffzusammensetzung ausmacht.

3. Verwendung nach Anspruch 1 oder Anspruch 2, bei der das Diisobutylen 5 Vol.% bis weniger als 15 Vol.% der gesamten Kraftstoffzusammensetzung ausmacht.

4. Verwendung nach einem vorhergehenden Anspruch, bei der das Diisobutylen eine Mischung von 2,4,4-Trimethylpent-1-en und 2,4,4-Trimethylpent-2-en umfasst.

5. Verwendung nach einem vorhergehenden Anspruch, bei der das Diisobutylen eine Mischung von 2,4,4-Trimethylpent-1-en und 2,4,4-Trimethylpent-2-en in einem Verhältnis von etwa 75 Gew.-% zu etwa 25 Gew.-% umfasst.

6. Verwendung nach einem vorhergehenden Anspruch, bei der der Basiskraftstoff Mischungen von gesättigten, olefinischen und aromatischen Kohlenwasserstoffen umfasst, die von Einfachdestillatströmen, thermisch oder katalytisch gecrackten Kohlenwasserstoffeinsatzmaterialien, durch Hydrocracken gewonnenen Erdölfraktionen, katalytisch reformierten Kohlenwasserstoffen oder synthetisch hergestellten Kohlenwasserstoffmischungen ableitbar sind.

7. Verwendung nach einem vorhergehenden Anspruch, bei der der Basiskraftstoff ein Erdölkraftstoff ist, der einen Siedebereich von Benzin, das typischerweise im Bereich zwischen 50 und 200 °C siedet und einen Endsiedepunkt von über 150 °C hat, bis zu Destillatkraftstoff aufweist, der typischerweise zwischen 150 und 400 °C siedet.

8. Verwendung nach einem vorhergehenden Anspruch, bei der der Basiskraftstoff ein herkömmlicher Destillatkraftstoff ist, der ausgewählt ist aus Motorbenzin, Kerosin und Dieselkraftstoffen.

9. Verwendung nach einem vorhergehenden Anspruch, bei der der Basiskraftstoff einen Schwefelgehalt von weniger als 100 Gew.-ppm hat.

10. Verwendung nach einem vorhergehenden Anspruch, bei der der Basiskraftstoff einen Schwefelgehalt von weniger als 50 Gew.-ppm hat.

## Revendications

1. Utilisation de diisobutylène comme agent anti-mousse pour un carburant de base ayant un point d'ébullition final supérieur à 150°C, dans laquelle le diisobutylène constitue plus de 2,5% en volume de la composition totale de carburant.

2. Utilisation selon la revendication 1, dans laquelle le diisobutylène constitue moins de 15% en volume de la composition totale de carburant.

3. Utilisation selon la revendication 1 ou 2, dans laquelle le düsobutylène constitue 5% à moins de 15% en volume de la composition totale de carburant.

4. Utilisation selon l'une quelconque des revendications précédentes, dans laquelle le düsobutylène comprend un mélange de 2,4,4-triméthylpent-1-ène et de 2,4,4-triméthylpent-2-ène.

5. Utilisation selon l'une quelconque des revendications précédentes, dans laquelle le diisobutylène comprend un mélange de 2,4,4-triméthylpent-1-ène et de 2,4,4-triméthylpent-2-ène dans un rapport d'environ 75% à environ 25% en poids.

6. Utilisation selon l'une quelconque des revendications précédentes, dans laquelle le carburant de base comprend des mélanges d'hydrocarbures saturés, oléfiniques et aromatiques qui peuvent être tirés de courants de première distillation, de charges d'hydrocarbures craquées par voie thermique ou catalytique, de fractions de pétrole hydrocraquées, d'hydrocarbures reformés par voie catalytique ou de mélanges d'hydrocarbures produits par synthèse.

7. Utilisation selon l'une quelconque des revendications précédentes, dans laquelle le carburant de base est un carburant de pétrole ayant une plage d'ébullition allant de l'essence (qui bout typiquement dans la plage de 50 à 200°C avec un point d'ébullition final dépassant 150°C) à un carburant de distillat (qui bout typiquement entre 150 et 400°C).

8. Utilisation selon l'une quelconque des revendications précédentes, dans laquelle le carburant de base est un carburant de distillat courant choisi parmi l'essence de moteur, le kerosène et les carburants diesel.

9. Utilisation selon l'une quelconque des revendications précédentes, dans laquelle le carburant de base a une teneur en soufre inférieure à 100 ppm en poids.

10. Utilisation selon l'une quelconque des revendications précédentes, dans laquelle le carburant de base a une teneur en soufre inférieure à 50 ppm en poids.
